

## UNITED STATES PATENT OFFICE

CLARENCE S. WICKES, OF MERCHANTVILLE, NEW JERSEY, ASSIGNOR TO VICTOR  
TALKING MACHINE COMPANY, A CORPORATION OF NEW JERSEY

## DIAPHRAGM

No Drawing.

Application filed December 7, 1925. Serial No. 73,902.

This invention relates to diaphragms and more particularly to diaphragms for use in reproducing sound.

Many substances have heretofore been employed for making sound reproducing diaphragms. For example, commercial aluminum has been suggested for making diaphragms for talking machine sound boxes. In order to employ materials of this nature it is necessary that the metal be rolled into extremely thin sheets, a thin, light diaphragm being desired for the reproduction of high frequency sound waves. For example, frequencies on the order of 5,000 are involved when it is desired to reproduce the highest note of an orchestra.

Difficulty is encountered in rolling commercial aluminum into thin sheets for use in making diaphragms due to the impurities therein. Moreover, holes frequently develop during the rolling process of the sheet which seriously affect the value of the latter as a diaphragm material. Commercial aluminum of the best grade contains from 0.18 to 0.40 per cent of iron and 0.29 to 0.40 per cent of silica, among other impurities. Because of these impurities it is extremely difficult to form a diaphragm of commercial aluminum which will reproduce the high frequency sound waves. The reproduction of high frequencies is essential in order that the quality characteristics determined by the high partials of low and medium register notes may be secured and also in order that the fundamentals of the high register may be faithfully reproduced.

It is recognized, however, that aluminum possesses many characteristics which render it highly useful as a diaphragm material, but in view of the difficulty heretofore experienced in securing a satisfactory diaphragm of this material, it has been proposed to substitute duralumin in place of aluminum. Considerable difficulty and expense, however, is involved in rolling duralumin to the thickness required for diaphragm material and such thin sheets of duralumin are exceedingly difficult to handle without fracture. I have discovered that the difficulties heretofore experienced from the use of commercial alumi-

num may be greatly diminished, if not eliminated, by employing aluminum which is in a substantially chemically pure state, and at the same time avoid much of the difficulty that has been experienced in the efforts to substitute duralumin as a diaphragm material for aluminum.

An object of the present invention is to provide a diaphragm formed of chemically pure aluminum whereby a diaphragm of exceedingly light weight and extreme thinness is secured which is capable of faithfully reproducing very high frequencies.

Other objects of the invention are to provide a high frequency diaphragm which may be inexpensively rolled; which is durable and not readily subject to corrosion, and which has a greater internal viscosity or resistance than diaphragms heretofore produced, such for example as those formed of duralumin; to provide a diaphragm with a less rigid outer periphery than those heretofore formed of commercial aluminum and duralumin; and to provide a diaphragm material wherein deeper fins may be pressed and which may be more readily seated in a mounting, such, for example, as a talking machine sound-box.

In accordance with the present invention, chemically pure aluminum, that is aluminum which is approximately 99.9 percent pure, is rolled into sheets in any suitable manner well known in the art, approximately 1/500 of an inch in thickness. This thickness may be varied, however, in accordance with the size or diameter of the diaphragm it is desired to produce. I have discovered that aluminum is capable of an increased efficiency as regards reproduction of high frequency sound waves, is more durable and can be rolled into thinner sheets more inexpensively and satisfactorily than materials heretofore employed, if in a substantially chemically pure state, which at the present state of the art may contain approximately 0.005 percent of iron, 0.005 percent of silicon, no silica, and approximately 0.007 percent of copper. As herein employed, the term "chemically pure aluminum" refers to such aluminum, for example, as is produced by the Hoopes process described in a paper "The Electrolytic

Refining of Aluminum" by F. C. Frary  
(Transactions of the American Electro-  
chemical Society, Vol. XLVII, 1925, p.  
275).

5 After being rolled into sheets of desired thickness, the sheets are cut in any suitable manner, as by punching, into shapes of the desired size, and may be pressed into any suitable form. For example, fins may be  
10 pressed into the diaphragm to strengthen the same and enable the diaphragm to be of reduced thickness in order to favor low register notes.

By my discovery, after a series of experiments, that improved results may be secured by the use of chemically pure aluminum, whereby said aluminum may be worked to a thinner sheet than has heretofore been secured, thus securing a lighter diaphragm and  
20 one which secures better high frequency register, the difficulty and expense incident to forming a diaphragm of duralumin is obviated. Moreover, a lighter diaphragm is secured which has greater internal viscosity or  
25 resistance than a commercial aluminum diaphragm or one formed of duralumin, and which is therefore not so susceptible to rattles as a diaphragm formed of the materials mentioned above. Moreover, the diminution  
30 in the impurities, although only a fraction of a percent, is productive of relatively large advantageous results which are entirely disproportionate to the change in actual composition.

35 From the above it will be seen that the use of chemically pure aluminum for forming diaphragms for talking machine sound boxes results in a diaphragm of increased efficiency, in that the range of frequencies that  
40 can be reproduced is greatly extended, while it is less fragile and less subject to corrosion than commercial aluminum or duralumin.

Moreover, the use of chemically pure aluminum, which is a softer substance than  
45 either commercial aluminum or duralumin, results in a decided saving in the rolling operation. It is to be expressly understood that the present invention is not limited to dia-  
phragms for talking machine sound boxes,  
50 and reference will be had to the appended claim for a definition of the limits of the in-  
vention.

What is claimed is:

55 A diaphragm for reproducing sound waves which is formed from a rolled sheet of aluminum that contains not more than two-tenths percent of impurities and having high internal resistance.

In testimony whereof I have signed this  
60 specification.

CLARENCE S. WICKES.